

# UNITED STATES PATENT OFFICE.

LOUIS ELSBERG, OF NEW YORK, N. Y.

## IMPROVED PROCESS FOR SOLIDIFYING PEAT.

Specification forming part of Letters Patent No. 44,520, dated October 4, 1864.

*To all whom it may concern:*

Be it known that I, LOUIS ELSBERG, of the city, county, and State of New York, have invented a new and useful Process for Solidifying Peat; and I do hereby declare that the following is a full, clear, and exact description of my said invention.

Peat in its natural state is saturated with water, which it is necessary to remove in order to enable it to be conveyed to distant markets and to render it suitable for fuel. The peculiar porous structure of the peat opposes the removal of the water by direct pressure, while the removal of it by drying is not only a tedious process, but generally leaves the article with a loose open structure, which unfits it for conveyance to distant markets.

The object of my invention is to enable the peat to be solidified rapidly at a low cost; and it consists of a process composed essentially of three operations, which are, first, the beating of the peat; second, the grinding of it to a pulp, and, third, the separation of the water from it by pressure. In fact, I have discovered by experiment that when peat is subjected to a heat of about the boiling-point of water—say 212°—a change takes place in the character of the vegetable fibers contained in it, their elasticity appearing to be destroyed, and the change is such that the mass is readily reducible by grinding to a pulp, from which the water can be readily expressed, leaving the material in a hard solid cake, of a density approaching that of coal.

My invention is not confined to the use of particular machinery, and it may be practiced with machines now used for other purposes.

The best mode with which I am acquainted of applying the heat to the peat is by subjecting it in a vat to the action of steam produced in a high-pressure steam-boiler and introduced by a perforated pipe into the bottom of the vat. The best machinery with which I am acquainted for the purpose of grinding it to a pulp is the ordinary pulping-engine used for the manufacture of paper. The best machinery with which I am acquainted for the purpose of expressing the water is the hydraulic pressure used for pressing the stearine in the manufacture of stearine candles and for similar purposes. In order to practice my in-

vention with such machinery, I introduce a perforated steam-pipe directly into the bottom of the vat of the pulping-engine and connect this perforated pipe with the steam-boiler by a pipe fitted with a valve or stop-cock to regulate the passage of steam, so that the peat can be heated and ground simultaneously. I charge the vat of the engine with crude peat and water in such proportions that the mixture is sufficiently thin to be acted upon by the engine, the quantity of water added depending upon the wetness of the peat used. I then permit the steam to enter from the steam-boiler and commence the grinding. The steam rapidly heats the mass to the boiling-point, and the grinding rapidly reduces the mass to pulp. As soon as the charge of peat approaches a state of uniform pulp water is introduced to wash it, the surplus water being withdrawn without the pulp, in the usual manner practiced with paper-pulp, by a rotating scoop-wheel covered with fine wire-gauze. The heating, grinding, and washing are continued until the mass is reduced to a uniform pulp and the water is colorless, the effect of the washing being the removal of any soluble matters with which the peat is mixed. The operation is then stopped, and the mass of pulp is drained of water as thoroughly as possible, first, by the operation of the scoop-wheel, and then by discharging it from the mill and permitting it to lie upon a wire-gauze floor, after which it is subjected to pressure. For this purpose it may be first pressed lightly in perforated iron cases lined with wire-gauze, the tops and bottoms of the cases being formed by the platens of the press. The cakes produced by the first pressure should then be pressed a second time with the utmost pressure to which the material is to be subjected, and the pressing operation should be performed in a press heated by steam, like those employed for hot-pressing cakes of stearine in the candle manufacture, the effect of which is to solidify the cakes, so that they approximate coal in hardness and weight. The solidified peat in this form may be transported to market as coal is and used for fuel in the same manner.

Having thus described the best mode with which I am acquainted of practicing my invention, I declare that I do not claim to be the in-

ventor of the operation of grinding peat, nor of discharging the water from it by pressure, nor of the machinery I have described for practicing my invention; but

What I claim as my invention, and desire to secure by Letters Patent, is—

The process of solidifying peat by the operations of heating, grinding, and pressure, substantially as set forth.

In testimony whereof I have hereunto set my hand.

LOUIS ELSBERG.

Witnesses:

WILLIAM ELMER,  
LEOPOLD JAROSLAWSKI.